

## UNITED STATES PATENT OFFICE

FREDERICK M. BECKET, OF NEW YORK, N. Y., ASSIGNOR TO ELECTRO METALLURGICAL COMPANY, A CORPORATION OF WEST VIRGINIA

## COATING METAL ARTICLES

No Drawing.

Application filed October 29, 1928. Serial No. 315,931.

- The invention relates to processes for modifying the surfaces of metal articles by cementation. Examples of processes of this type are those known commercially as "sherardizing", "calorizing", and "chromizing". In a process covered in my Patent No. 1,672,444, dated June 5, 1928, both silicon and chromium are introduced into the surface of a metal article to form a corrosion-resistant layer. The present invention is especially adapted to be used in connection with the process of that patent, but it is applicable to other coating or casing processes of the cementation type.
- In cementation coating processes it is customary to incorporate into the cementation mixture a fluxing substance designed to expedite and regulate the formation of the desired coating. Such fluxing substances are sometimes called "energizers". Ammonium chloride has been widely and successfully used for this purpose. Zinc chloride has also been used.
- I have discovered that the use of a silicofluoride or fluosilicate as an energizer, for example the sodium salt,  $Na_2SiF_6$ , gives superior results, especially where silicon is to be incorporated into the surface coating. The silicofluoride gives a high rate of migration, and as compared with known energizers it often gives a denser and more coherent coating with a smoother and more uniform surface. At the higher cementation temperatures, ammonium chloride, zinc chloride and like energizers volatilize rapidly, displacing the cementation mixture with the result that contact is destroyed between the mixture and the article under treatment, and oxidizing gases, if present, are permitted to penetrate the mixture and to act on the surface to be coated. The silicofluorides, on the contrary, are practically non-volatile at the temperatures involved, and hence avoid the difficulties just described.
- The use of a silicofluoride energizer re-
- quires no change with respect to the other constituents of the mixture. Excellent results have been had using a mixture containing powdered iron-chromium-silicon alloy 55 parts; alumina 45 parts; and sodium silicofluoride 2.5 parts. The alloy contained approximately Cr 40% and Si 20%. As in the case of other energizers the action of the silicofluoride is analogous to that of a catalyst, and the proportion used is not a matter of great importance. Merely by way of example it may be stated that a proportion of silicofluoride between 0.5% and 10% is suitable, but a useful effect can undoubtedly be obtained with a content outside this range.
- In the appended claims, the term "metal" designates a substance having metallic characteristics and containing one or more chemical elements. Silicon for the purposes of this application, is classified as a metal. Where the claims recite silicon as a constituent of a cementation mixture, it will be understood that so-called metallic silicon or its alloys or silicides is meant.
- I claim:—
1. A cementation mixture comprising a silicofluoride and a corrosion-resisting metal.
  2. A cementation mixture comprising a silicofluoride and silicon.
  3. A cementation mixture comprising a silicofluoride and an alloy containing chromium and silicon.
  4. A cementation mixture comprising 0.5% to 10% of sodium silicofluoride and an alloy containing iron, chromium and silicon.
  5. The process of forming a coating on a ferrous article which comprises heating the article in contact with a mixture containing a silicofluoride and a corrosion-resisting metal until cementation occurs.
  6. The process of forming a coating on a ferrous article which comprises heating the article in contact with a mixture containing a silicofluoride and silicon until cementation occurs.

7. The process of forming a coating on a ferrous article which comprises heating the article in contact with a mixture containing a silicofluoride and an alloy containing chromium and silicon until cementation occurs.

8. The process of forming a coating on a ferrous article which comprises heating the article in contact with a mixture containing a silicofluoride and an alloy containing iron, chromium and silicon until cementation occurs.

In testimony whereof, I affix my signature.  
**FREDERICK M. BECKET.**

**15****20****25****30****35****40****45****50****55****60****65**